

## UNITED STATES PATENT OFFICE

2,231,446

## TREATMENT OF HYDROCARBONS

Aristid V. Grosse, Chicago, Ill., assignor to Universal Oil Products Company, Chicago, Ill., a corporation of Delaware

No Drawing. Application April 14, 1937,  
Serial No. 136,897

7 Claims. (Cl. 260—677)

This invention relates particularly to the treatment of hydrocarbons for the dehydrogenation thereof and is applicable to the treatment of any type of hydrocarbons containing more hydrogen than aromatics to produce more highly unsaturated derivatives either by simple dehydrogenation or dehydrocyclization reactions.

In a more specific sense the invention is concerned with a process employing specific types of catalysts and specific types of containers for said catalysts which are constructed of metals having substantially no direct influence upon the course of the dehydrogenation reactions so that the reactions may be better controlled and the life of the catalysts extended.

It has been shown by extensive experiments that the course of dehydrogenation reactions involving for example the production of mono olefins from paraffins, the production of diolefins from mono olefins, the formation of aromatics by the dehydrogenation and subsequent cyclization of aliphatic hydrocarbons can be influenced in the direction of greater selectivity by the use of proper catalysts so that the formation of undesirable by-products corresponding to secondary reactions is kept at a practical minimum. In large scale operations, however, it has been found that as a rule adverse influences are exerted on the course of these reactions by the ordinary materials of construction including ordinary steels and also special alloy steels comprising the elements cobalt, nickel, and chromium. In the case of steel tubes which contain dehydrogenating catalysts, there is a pronounced tendency for carbon to deposit where the hydrocarbon stream contacts the steel so that not only is the real catalyst contaminated but difficulties arise in temperature control on account of the insulating effect of the carbon film. These difficulties are of course obviated if tubes of ceramic material or silica are employed, but these materials are fragile and in general not adapted to service when pressures either above or below atmospheric are employed on account of the difficulty of properly cementing or packing joints to prevent leakage.

In one specific embodiment the present invention comprises the use of aluminum-bronze alloys as containers for granular dehydrogenating catalysts comprising relatively inert supporting materials having deposited thereon minor percentages of oxides of elements in the left-hand columns of the fourth, fifth and sixth groups of the Periodic Table.

It has been shown that aluminum bronzes have substantially no influence upon the course of hydrocarbon dehydrogenation reactions and furthermore that they have no influence upon the action of the catalysts which will presently be described in more detail. The term "aluminum bronze" as used in the present connection refers to alloys which contain as their essential components aluminum and copper with perhaps minor traces of iron and other elements. This definition is given to distinguish the present type of materials from those which might contain definite quantities of other elements such as those which contain as high as 3% iron and those which contain tin as well as copper and still fall under the definition of bronze. Materials of the present character can be worked into tubes and chambers of considerable size and the alloys themselves have sufficient tensile strength to permit the use of subatmospheric and moderately superatmospheric pressures at temperatures of the order of 450–650° C. which include most of those used in connection with the preferred hydrogenating catalysts. It is also within the scope of the invention to employ steel tubes which have been properly lined by aluminum-bronze alloys.

The dehydrogenating catalysts which are employed in aluminum bronze tubes in accordance with the present invention comprise a particular group of composite catalytic materials which employ as supporting materials certain refractory oxides which in themselves may have some slight specific catalytic ability in dehydrogenation reactions but which are improved greatly in this respect by the addition of certain promoters or secondary catalysts in minor proportions. These supporting materials are preferably of a rugged and refractory character capable of withstanding the severe use to which the catalysts are put in regard to temperature during service and in regeneration by means of air or other oxidizing gas mixtures after they have become fouled with carbonaceous deposits after a period of service. The preferred supporting materials comprise oxides of aluminum and magnesium oxide.

The magnesium and aluminum oxides mentioned may be considered as base catalytic materials which may have some slight specific dehydrogenating action in themselves but which are improved materially in this respect by the addition of more catalytically active promoters. Either of these oxides may be prepared by the controlled calcination of either suitable ores or

minerals or chemically prepared compounds which yield the oxides on ignition. As a general rule magnesium oxide is most conveniently prepared from the mineral magnesite and aluminum oxide is similarly available by the ignition of bauxite having the formula  $Al_2O_3 \cdot 2H_2O$ . The mineral diaspore having the formula  $Al_2O_3 \cdot H_2O$  does not furnish a sufficiently good type of aluminum oxide after calcination for use in the present instance. In the paragraphs immediately following, some space will be devoted to these base materials and their preferred modes of preparation.

Magnesium oxide itself prepared by the controlled calcination of natural magnesite is in itself a fairly good catalyst for accelerating the rate and controlling the character of dehydrogenating reactions over a considerable tempera-

$Na_2Al(CO_3)_3$ , an alkalinized aluminum oxide is preparable directly.

The promoters which are used on the supporting materials include preferably oxides of certain elements which occupy what may be termed a definite area in the periodic table, and which therefore may be classed as a natural group. The elements whose oxides have been found to exert the best catalytic effects in paraffin dehydrogenation reactions are those in the lefthand columns of groups 4, 5, and 6, and for indicating these elements and their relative positions the following tabulation is introduced which is an abbreviated section of the periodic table of the elements as at present accepted. The table also includes the elements in the right-hand columns, though these are not included as sources of catalysts according to the present invention.

20

| Group IV                                |                      | Group V                                          |                         | Group VI                                         |                           |
|-----------------------------------------|----------------------|--------------------------------------------------|-------------------------|--------------------------------------------------|---------------------------|
| Left                                    | Right                | Left                                             | Right                   | Left                                             | Right                     |
| <u>Titanium</u><br>Zirconium<br>Hafnium | (Germanium)<br>(Tin) | <u>Vanadium</u><br><u>Columnbium</u><br>Tantalum | (Arsenic)<br>(Antimony) | <u>Chromium</u><br><u>Molybdenum</u><br>Tungsten | (Selenium)<br>(Tellurium) |

20

25

ture range. However, an extensive series of experiments has demonstrated that this catalytic property is greatly improved by the addition of certain promoting substances in minor amounts, usually in the order of less than 10% by weight of the oxide.

The mineral magnesite is most commonly encountered in a massive or earthy variety and rarely in crystal form, the crystals being usually rhombohedral. In many natural magnesites, the magnesium oxide may be replaced to the extent of several per cent by ferrous oxide. The mineral is of quite common occurrence and readily obtainable in quantity at a reasonable figure. The pure compound begins to decompose to form the oxide at a temperature of  $350^{\circ} C.$ , though the rate of decomposition only reaches a practical value at considerably higher temperatures, usually of the order of  $800^{\circ} C.$  to  $900^{\circ} C.$  Magnesite is related to dolomite, the mixed carbonate of calcium and magnesium, the latter mineral, however, not being of as good service as the relatively pure magnesite in the present instance. Magnesium carbonate prepared by precipitation methods may also be employed as a source of magnesium oxide with any type of activation which may be employed to produce a material of good porosity and structural strength.

Aluminum oxide to be used as a carrier for the preferred metal oxide catalysts may be prepared by the ignition either of precipitated aluminum hydroxide or by ignition of such natural minerals as bauxite as already mentioned. The ignited aluminum oxide which is apparently in best physical condition for catalytic use when temperatures of approximately  $600$ – $750^{\circ} C.$  have been employed may be "alkalized" by small amounts of alkali metal or alkaline earth metal hydrates or carbonate, which seems to extend the life of the finally prepared catalyst composite possibly on account of a slower rate of carbon deposition. These alkalized materials have been found to be more easily regenerated when the carbonaceous deposits are removed by air or other oxidizing gas mixture. By ignition of the mineral dawsonite having the formula

The elements given above whose oxides are preferred as dehydrogenating catalysts according to the present invention are apparently further characterized by a variation in catalytic effectiveness in a horizontal direction and are also characterized by the fact that in general the most effective catalysts are oxides of elements which are most readily oxidizable and reducible. Thus in a general way the effectiveness of the catalysts increases from Group IV to Group VI and decreases in Group VI downwardly. There are some irregularities in these characterizations, particularly in regard to compounds of vanadium which are particularly efficient catalysts, although the oxides of vanadium are not the most easily reducible of the preferred elements of Groups IV and V.

Catalyst composites comprising supporting materials of the types indicated and oxides of the elements shown may be prepared by utilizing certain soluble compounds of the elements in aqueous solutions from which they are absorbed by prepared granular carriers or from which they are deposited upon the carriers by evaporation of the solvent. In order to promote complete adsorption of the salts the solutions may be concentrated by evaporation in the presence of the adsorbent material or even evaporated to complete dryness in some cases. In the latter case it is obvious that good distribution of the promoting material will be assisted by thorough mixing during the drying period.

The most general method for adding the preferred oxide catalyst to the supporting materials (which if properly prepared have a high adsorptive capacity) is to stir prepared granules of from approximately 4 to 20 mesh into solutions of salts which will yield the desired promoting compounds on ignition under suitable conditions, such as the nitrates, in some instances the sulfates, and in other instances acids corresponding to the hydrated oxides, for example, chromic acid in the case of chromium. In some instances the granules may be merely stirred in slightly warm solutions of salts until the dissolved compounds have been retained on the particles by absorp-

30

35

40

45

50

55

60

65

70

75

75

tion or occlusion, after which the particles are separated from the excess solvent by settling or filtration, washed with water to remove excess solution, and then ignited to produce the desired residual promoter. In cases of certain compounds of relatively low solubility it may be necessary to add the solution in successive portions to the adsorbent base catalyst with intermediate heating to drive off solvent in order to get the required quantity of promoter deposited upon the surface and in the pores of the base catalyst. The temperatures used for drying and calcining after the addition of the promoters from solutions will depend entirely upon the individual characteristics of the compound added and no general ranges of temperature can be given for this step.

Catalytic promoters may be added to the supports by precipitating the hydroxides of certain elements onto the granular supports suspended in aqueous solution, by adding alkali hydroxides, aluminum hydroxide or the corresponding carbonates. The occluded hydroxides are then calcined at suitable temperatures for producing the corresponding oxides. Experience has shown that it is better to subject the oxides to a reducing action before employing the catalyst composites in dehydrogenating reactions since evidently the best catalytic effects are accomplished by the lower oxides such as the sesquioxide  $\text{Cr}_2\text{O}_3$  in the case of chromium and the corresponding oxide  $\text{V}_2\text{O}_3$  in the case of vanadium. If this is not done there is usually an "induction period" in which the catalyst is gradually reduced to its lower valence by the hydrocarbon vapors passing over it.

In regard to the relative proportions of supports and catalysts it may be stated in general that the latter are generally less than 10% by weight of the total composites. The effect upon the catalytic activity of the composite caused by varying the percentage of any given oxide deposited thereon is not a matter for exact calculation but more one for determination by experiment. Frequently good increases in catalytic effectiveness are obtainable by the deposition of as low as 1% or 2% of a promoting compound upon the surface and in the pores of the base catalyst, though the general average is about 5%.

Dehydrogenating catalysts of the character described may be used over a considerable range of temperatures and pressures and hydrocarbons to be dehydrogenated more or less extensively may be contacted with the catalytic materials for widely varying times. In general the temperatures vary from 400-700° C., pressures from about 0.25 atmospheres absolute to superatmospheric of the order of 100 lbs. per square inch and times from 0.1 to as high as 50 seconds.

When paraffins are dehydrogenated to the corresponding mono olefins temperatures of the order of 500-600° C., atmospheric or slightly superatmospheric pressures and times of contact up to 6 seconds are usually adequate. When using the same catalysts to produce diolefins from mono olefins the same general range of temperatures are applicable but best results are usually obtained with subatmospheric pressures of the order of 0.25 atmospheres and relatively short times of contact, commonly less than 1 second. When dehydrogenating aliphatic hydrocarbons with the object of producing aromatic hydrocarbons by successive dehydro- and cyclization reactions, the temperatures may be raised to points approaching the upper limit of 700° C. and the

times of contact may be extended to as high as 50 seconds depending upon the hydrocarbon undergoing treatment though as a rule times of from 15-20 seconds are adequate. These approximate ranges are merely given to indicate that considerable variation in operating conditions may be employed.

Any of the alternative catalysts prepared by the previously described methods may be pre-treated if desired by any necessary method at elevated temperatures to increase their activity. In the heat treatment gases such as air, steam, carbon dioxide, hydrogen, nitrogen, etc. are passed over the catalyst particles at elevated temperatures. No general rule can be laid down for the temperature and time necessary to activate the catalysts, the best activating temperature sometimes being higher and sometimes lower than the optimum temperature at which they may be employed for treatments. The use of hydrogen or other reducing gas mixture prior to putting the catalyst in service will usually eliminate an induction period corresponding to the time necessary to reduce the oxides to those of lower valence, which are apparently the active catalysts.

The following illustrative data are introduced to show the improved results obtainable when employing aluminum bronze tubes instead of steel tubes or even certain special alloys in current use although the scope of the invention is not to be exactly limited to the data presented.

Using a catalyst comprising approximately 95% by weight of an activated alumina supporting 5% by weight of chromium sesquioxide, runs 35 were made to dehydrogenate a mixture of butanes to produce a mixture of butenes. When a steel tube was employed as a catalyst container the carbon formation at 500° C. and atmospheric pressure was very rapid so that the tube became 40 plugged with carbon in a few hours' operation. Using a tube of nickel-chromium-steel the operation was improved to the extent that a run of 250 hours was possible before carbon deposition rendered continuing the process impractical. 45 When an aluminum-bronze tube having a composition of approximately 10% aluminum and 90% copper was employed, there was substantially no carbon deposits after a period of 1000 hours' operation which indicates the marked 50 superiority of this type of material over those in common usage in hydrocarbon conversion reactions.

The nature of the invention is evident from the preceding specification and the numerical 55 data although neither section is intended to be unduly limiting upon those generally broad in scope.

I claim as my invention:

1. A process for the catalytic dehydrogenation 60 of hydrocarbons which comprises subjecting said hydrocarbons at temperatures of the order of 400-700° C. to contact with dehydrogenating catalysts in containers whose inner surfaces exposed to the hydrocarbons and catalyst are composed of an alloy consisting essentially of aluminum and copper and substantially free of iron and tin.

2. A process for the catalytic dehydrogenation 70 of normally gaseous hydrocarbons which comprises subjecting said hydrocarbons at temperatures of the order of 400-700° C. to contact with dehydrogenating catalysts in containers whose inner surfaces exposed to the hydrocarbons and catalyst are composed of an alloy consisting es- 75

sentially of aluminum and copper and substantially free of iron and tin.

3. A process for the catalytic dehydrogenation of hydrocarbons of approximate gasoline boiling range which comprises subjecting said hydrocarbons at temperatures of the order of 400-700° C. to contact with dehydrogenating catalysts in containers whose inner surfaces exposed to the hydrocarbons and catalyst are composed of an alloy consisting essentially of aluminum and copper and substantially free of iron and tin.

4. A process for the catalytic dehydrogenation of hydrocarbons which comprises subjecting said hydrocarbons at temperatures of the order of 400-700° C. to contact with dehydrogenating catalysts comprising essentially relatively inert granular materials supporting less than 10% by weight of oxides of elements in the lefthand columns of groups IV, V, and VI of the periodic table in containers whose inner surfaces exposed to the hydrocarbons and catalyst are composed of an alloy consisting essentially of aluminum and copper and substantially free of iron and tin.

5. A process for the catalytic dehydrogenation of normally gaseous hydrocarbons which comprises subjecting said hydrocarbons at temperatures of the order of 400-700° C. to contact with dehydrogenating catalysts comprising essentially relatively inert granular materials supporting less than 10% by weight of oxides of elements in the lefthand columns of groups IV, V, and VI of the periodic table in containers whose inner surfaces exposed to the hydrocarbons and catalyst are composed of an alloy consisting essentially of aluminum and copper and substantially free of iron and tin.

periodic table in containers whose inner surfaces exposed to the hydrocarbons and catalyst are composed of an alloy consisting essentially of aluminum and copper and substantially free of iron and tin.

6. A process for the catalytic dehydrogenation of hydrocarbons of approximate gasoline boiling range which comprises subjecting said hydrocarbons at temperatures of the order of 400-700° C. to contact with dehydrogenating catalysts comprising essentially relatively inert granular materials supporting less than 10% by weight of oxides of elements in the lefthand columns of groups IV, V, and VI of the periodic table in containers whose inner surfaces exposed to the hydrocarbons and catalyst are composed of an alloy consisting essentially of aluminum and copper and substantially free of iron and tin.

7. A process for the catalytic dehydrogenation of hydrocarbons which comprises subjecting said hydrocarbons at temperatures of the order of 400-700° C. to contact with dehydrogenating catalysts comprising essentially aluminum oxide supporting less than 10% by weight of the oxides of the elements in group VI of the periodic table in containers whose inner surfaces exposed to the hydrocarbons and catalyst are composed of an alloy consisting essentially of aluminum and copper and substantially free of iron and tin.

ARISTID V. GROSSE.